

(No Model.)

W. S. PLATT.

METHOD OF MAKING ELECTRICAL CONDUCTORS.

No. 320,684.

Patented June 23, 1885.

Fig. 1



Fig. 2



Fig. 3



Witnesses

S. Williamson  
Harry T. Stephens.

Inventor

William S. Platt  
Smith & Hubbard  
Atty's.

# UNITED STATES PATENT OFFICE

WILLIAM S. PLATT, OF WATERBURY, CONNECTICUT.

## METHOD OF MAKING ELECTRICAL CONDUCTORS.

SPECIFICATION forming part of Letters Patent No. 320,684, dated June 23, 1885.

Application filed May 15, 1884. (No model.)

*To all whom it may concern:*

Be it known that I, WILLIAM S. PLATT, a citizen of the United States, residing at Waterbury, in the county of New Haven and State 5 of Connecticut, have invented certain new and useful Improvements in Electrical Conductors; and I do hereby declare the following to be a full, clear, and exact description of the invention, such as will enable others skilled in the 10 art to which it appertains to make and use the same.

My invention relates to certain novel and useful improvements in the manufacture of electrical conductors for long distances; and 15 has for its object to provide such a device which shall be exceedingly simple in its construction, while at the same time a firm union between the component parts is established, and the conductor rendered durable and positive; and with these ends in view my invention 20 consists in the details of construction and combination of elements hereinafter fully and in detail explained, and then specifically designated by the claim.

25 In order that those skilled in the art to which my invention appertains may more fully understand its construction and adaptation, I will proceed to describe the same, referring by letter to the accompanying drawings, forming 30 a part of this specification, in which—

Figure 1 is a perspective view illustrating my improvement; Fig. 2, an end view showing the copper sheath secured to the core by means of a lock-seam extending within the 35 channel, and Fig. 3 a modification showing the edges of the sheath of copper or other suitable material abutting against each other.

Similar letters denote like parts in the several figures of the drawings.

40 A is a central core of steel which is fluxed and run through a bath of solder, and B a sheath or envelope of copper or any other suitable material, which is curled around the core after the latter has come out of the solder bath. The edges of the copper overlap one 45 above the other, the lower edge being swaged and forced within a concave channel, C, in the core A.

In the drawings, Fig. 1, D represents the 50 solder, which extends entirely around the core, so that the copper sheath is firmly united there-

to. The peculiar manner shown of overlapping the edges of the sheath prevents the latter from turning on the core, if it is ever dis-united therefrom. At Fig. 2 I have shown the 55 said edges united by a lock-seam, and at Fig. 3 I have shown the sheath of copper drawn around a cylindrical core, and with the edges abutting and not overlapping.

By careful examination it will be seen that 60 the circular channel in the steel core must be proportionate in depth and width to the extent of the lap in the covering, and also to the thickness of the covering; hence if the proportion of copper to the steel needs to be increased for conductivity the channel may be widened and deepened and the overlap increased accordingly. This enables me to have a larger portion of copper, with the advantage 65 of a lock-seam, avoiding the use of solder in 70 some cases.

One of the distinctive features of my invention is the channel in the steel core, since by this arrangement I am enabled to make a simple lap without scarfing, and a lock-seam of 75 great firmness and still retain the cylindrical form of the exterior.

In adapting the copper sheath to the steel core, as shown at Fig. 1, I proceed as follows: The steel core, properly prepared with a flux 80 composed of a sal ammoniac solution or zinc chloride, or both, and then dried, is run through a bath of solder. Then the above-named fluxing is repeated upon the surface of the solder, and a copper sheath drawn or 85 curled around the same, the edges of said sheath being overlapped and forced within the channel in the core, as previously set forth. The parts are then subjected to the action of heat, and then passed through dies which compress 90 the sheath and core firmly together, and a cooling agent applied which causes the solder to unite their contact-surfaces.

I am enabled to produce similar results by fluxing the inner surface of the copper sheath 95 instead of the solder surface, and do not wish to be limited in this respect.

I am aware that a conductor composed of steel with a copper sheath is not new, broadly; and I do not wish to be understood as laying 100 claim to any such construction, the gist of my invention lying in the peculiar method of unit-

ing these metals either by solder or by a lock-seam.

Having thus described my invention, what I claim as new, and desire to secure by Letters 5 Patent, is—

The method herein described of making electrical conductors, the same consisting in providing a core of iron or steel, having in its face a longitudinal channel, then enveloping said core with a sheath of copper or other suitable

material, the edges of said sheath being overlapped and forced within said channel, substantially as set forth.

In testimony whereof I affix my signature in presence of two witnesses.

WILLIAM S. PLATT.

Witnesses:

CLARK M. PLATT,  
D. F. WEBSTER.